

# UNITED STATES PATENT OFFICE.

ALVAH W. CLEMENT, OF EAST CLEVELAND, OHIO, ASSIGNOR TO THE CLEVELAND  
BRASS MANUFACTURING COMPANY, OF CLEVELAND, OHIO, A CORPORATION  
OF OHIO.

## ALLOY.

1,400,527.

Specification of Letters Patent. Patented Dec. 20, 1921.

No Drawing.

Application filed July 21, 1917. Serial No. 182,005.

To all whom it may concern:

Be it known that I, ALVAH W. CLEMENT, a citizen of the United States, residing at East Cleveland, in the county of Cuyahoga and State of Ohio, have invented a certain new and useful Improvement in Alloys, of which the following is a full, clear, and exact description.

Iron in the various forms in which it is commercially known and used is not effectively resistant to oxidization and warping when repeatedly subjected to heatings to high temperatures, and iron containers, saggars, pyrometer tubes, and other structural forms of iron when so repeatedly heated, deteriorate quite rapidly.

Nevertheless, iron because of its properties of easy machinability, ease of casting and accessibility at comparatively low price, has been the metal chiefly used for such purposes before mentioned.

This invention has for its object, the provision of a metal alloy which is highly resistant to oxidization and warping, and generally effectively withstands deterioration when subjected to repeated heatings to high temperature. Furthermore, the alloy is easily machined and may readily be cast.

The alloy of this invention includes as constituent elements, chromium, iron, silicon and aluminum, and optionally vanadium.

The chromium imparts to the alloy the property of resistance to warping even when repeatedly heated to high temperatures.

Silicon imparts to the alloy the property of resistance to oxidization when heated to high temperatures under oxidizing conditions.

Aluminum gives the metal a good grain structure.

Vanadium when used, increases the tensile strength although the alloy without the addition of vanadium is very satisfactory in this respect.

There is, of course, some carbon present in the alloy, and may be in the combined state as a carbide of iron and chromium, or it may be in the free state as graphitic carbon, or it may be present in both conditions.

If the alloy in its use is to be subjected to fumes of sulfurous or sulfuric acid, the alloy is more resistant to such fumes when the carbon is in the combined form. On the other

hand, the alloy is more resistant to the fumes of nitric acid or acids of this group, when the carbon is in the uncombined condition.

The proportions of the various elementary constituents may vary, some within rather wide range, while others may not.

For instance, chromium when forming from 20% to 40% of the alloy, imparts to the alloy the property of nonwarping at high temperatures. However, the most desirable and effective proportion of chromium is from 30% to 35% of the alloy.

Silicon is advantageously used only in small quantities, *i. e.* from 1% to 2%. Increasing the proportion of silicon makes the alloy more grainy, thus affecting the tensile strength and cross grain strength.

Aluminum is desirable only in small proportion from  $\frac{1}{2}$  of 1% to 1%. Aluminum is rather readily oxidizable, especially at high temperatures under oxidizing conditions.

The carbon content of the alloy is very low. In fact, it is made as low as possible, for the effect of the carbon is to work against the chromium and neutralizes its non-warping properties.

When vanadium is used, it forms only  $\frac{1}{2}$  of 1% to 1% of the alloy.

The iron is always the preponderating element in the alloy, making up the remaining proportion of the alloy when the other ingredients are employed in the proportions mentioned.

This alloy is very high in tensile strength, and has a good fracture on cross breaking.

It has a low coefficient of expansion and has no growth upon repeated heatings and coolings.

It is easily machined and drilled, and may readily be cast.

The grain of the alloy is dense, and is not affected by the oxyhydrogen or oxyacetylene flame.

The most important and dominant features of the alloy are those early mentioned in the specification, to-wit non-warping and resistance to oxidization when repeatedly heated to high temperatures even under oxidizing conditions.

In speaking of high temperatures which the alloy may withstand, reference is to temperatures of from 2000° Fah. to substantially 2500° Fah.

A notable feature of the alloy is that thin walled structures effectively withstand warping, so that light structures may be employed for any particular work, obviating clumsiness or excessive weight.

It will be clear from the foregoing that the fusion point of the alloy is quite high, and so far as known, only in the electric furnace can sufficient heat be gotten to produce 10 fusion.

Having thus described my invention, what I claim is:

1. A metallic alloy which is substantially non-warping and resistant to deterioration 15 when heated to high temperature containing iron, chromium in excess of 10% and a small quantity of silicon and aluminum.

2. A metallic alloy which is substantially non-warping and resistant to deterioration 20 when heated to high temperature, containing essentially iron, chromium in excess of 10% and another substance having the properties of silicon which resists oxidization at high temperature.

25 3. A metallic alloy which is substantially non-warping and resistant to deterioration when heated to high temperature containing essentially iron and chromium in excess of

10%, and a sufficient amount of silicon to resist oxidization at high temperature.

4. A metallic alloy which is substantially non-warping and resistant to deterioration when heated to high temperature containing essentially iron and chromium in excess of 30 10%, and not more than 2 per cent. of silicon and not more than 1 per cent. of aluminum.

5. A metallic alloy which is substantially non-warping and resistant to deterioration 35 when heated to high temperature containing essentially iron and a small quantity of chromium, in excess of 10% silicon and aluminum, and less than 1 per cent. of carbon.

6. A metallic alloy containing 20 to 40 40 per cent. of chromium, 1 to 2 per cent. of silicon,  $\frac{1}{2}$  to 1 per cent. of aluminum, and the remainder iron.

7. A metallic alloy containing 20 to 40 45 per cent. of chromium, 1 to 2 per cent. of silicon,  $\frac{1}{2}$  to 1 per cent. of aluminum, substantially  $\frac{1}{2}$  of 1 per cent. of vanadium, and the remainder iron.

In testimony whereof, I hereunto affix my signature.

ALVAH W. CLEMENT.